

Patented Aug. 13, 1929.

1,724,552

# UNITED STATES PATENT OFFICE.

ARTHUR E. BELLIS, OF BRANFORD, CONNECTICUT.

## SALT BATH.

No Drawing. Original application filed September 10, 1925, Serial No. 55,623. Divided and this application filed March 18, 1929. Serial No. 348,145.

This invention relates to salt baths such as are used for the heat treatment of metals and other purposes, and constitutes a division of my pending application Serial No. 5 55,623, filed September 10, 1925.

In general, the invention has for its primary object and purpose to provide a salt bath composition containing in solution therewith a scavenging agent acting as a solvent for oxides and other impurities carried into the bath with the metal or entering the bath from the crucible wall, and thereby preventing contamination of the bath and maintaining the same at all times 10 chemically neutral to the metal.

It is also an important object of the invention to provide such a salt bath composition containing the automatically acting scavenging ingredient which will possess 20 maximum stability, high heat transfer efficiency and which will provide an ideal heating curve for the metal. In addition, the new bath is easily controllable as to the melting point of its components within an appreciable temperature range, whereby its 25 viscosity may be regulated or varied without effect upon its neutrality to the chemical composition of the metal being treated.

Generically, the invention comprehends 30 the use in such a salt bath for the heat treatment of metals of a boron compound and an alkaline chloride.

In the heat treatment of metals by immersion in a salt bath, of the eutectic single phase or the non-eutectic multi-phase type, I have succeeded in developing a bath composition which, even after excessive heating at high temperatures, is automatically maintained entirely free of contamination by impurities such as metallic oxides. Specifically, the bath hereinafter referred to is primarily designed and intended for use in the hardening of high speed tool steels or alloys, and which bath must remain stable and 45 without appreciable volatilization at temperatures up to 2500° F. I have succeeded in accomplishing this result by using in solution with the bath, an alkaline salt together with a boron salt, the latter constituting a 50 solvent for practically all oxides (as of Na, K, Ba, Fe, etc.) which fuse with the boron salt to give borates. In a preferable embodiment of the invention, I utilize a compound boron salt preferably consisting of boron trioxide ( $B_2O_3$ ) and sodium meta borate 55 ( $NaBO_2B_2O_3$ ). I have found in practice that the use of such a boron compound with an alkaline chloride in either a eutectic or non-eutectic salt bath, will act automatically as a solvent for any oxides or other impurities entering the bath solution and maintain the original single or multi-phase character of the bath solution. 60

I preferably employ as an alkaline salt, potassium chloride, though if desired, potassium nitrate or any other alkaline salt may be substituted. 65

In practice I have found that a salt bath having the above characteristics, may be successively used in the heat treatment of 70 high speed tool steels or alloys, and in contra-distinction to a bath of commercial borax, will not deleteriously or harmfully effect the metal, as by pitting the metal surface or decarburization of the metal. Such 75 harmful effects are usually caused by the presence of undissolved metallic oxides in the bath solution. These oxides also very seriously affect the uniformity in the rate of heating of the metal piece as well as reacting chemically therewith to cause decarburization. By my new bath employing the boron compound as an automatically acting solvent for such oxides, a clear 80 homogeneous solution is maintained at all 85 times and the viscosity of the solution remains constant so that the rate of heat transfer through the solution to the metal immersed therein is invariable. This rate of heat transfer may however, be easily controlled and regulated by either increasing 90 or decreasing the proportion of the borates in the bath which changes its viscosity, and thus enables the metal to be treated through a desired temperature range. From the 95 above, it will be apparent that my new bath solution provides a metal heat treating medium whereby uniformly successful results may be attained in the heat treatment of high speed tool steels or alloys owing to 100 the entire absence of undissolved metallic oxides in the bath. Therefore, the bath is maintained in a stable condition and its tendency to decompose or undergo changes 105 in composition due to chemical reaction with such oxides is eliminated. Also the protective action of the bath film adhering to the surfaces of the metal when it is withdrawn from the solution is greatly improved. 110

I preferably use in connection with the high temperature bath above described, a quenching bath which consists of a eutectic mixture of potassium chloride and sodium carbonate which I have found to be particularly applicable and desirable in the heat treatment of high carbon content high speed steel or alloy.

It will be understood that the relative proportions of the two boron constituents of the potassium salt may be varied in order to secure the desired viscosity of the bath solution. As an example however, of a specific composition which I have successively used, I may refer to a bath solution containing substantially 31% of boron trioxide, 49% of sodium meta borate, and 20% of potassium chloride. In this example, I have stated the proportionate quantities of the salt components before fusion, and it is possible that in the fusion of said components, certain complex salts may be formed and that, therefore, the fused mixture upon analysis, would not be found to contain the said components in the exact original proportions. It is however, unnecessary to consider such complex salts as may be formed in the bath solution since

I have found that the characteristics of the bath solution as above referred to are not materially affected.

I claim:

1. A stable high temperature salt bath for heat treating metals containing boron trioxide as an oxide solvent.
2. A stable high temperature salt bath for heat treating metals containing in solution boron trioxide and sodium meta borate as an oxide solvent.
3. A high temperature salt bath for heat treating metals consisting of a stable homogeneous solution containing boron trioxide and an alkaline chloride.
4. A high temperature salt bath for heat treating metals consisting of a stable homogeneous solution containing boron trioxide, sodium meta borate, and an alkaline chloride.
5. A high temperature salt bath for heat treating metals consisting of a stable homogeneous solution containing boron trioxide, sodium meta borate, and potassium chloride.

In testimony that I claim the foregoing as my invention, I have signed my name hereto.

ARTHUR E. BELLIS.